

# UNITED STATES PATENT OFFICE.

LEWIS B. LINDEMUTH, OF STEELTON, PENNSYLVANIA.

## METHOD OF MAKING SOUND STEEL CASTINGS.

Specification of Letters Patent. Patented Nov. 10, 1914.

1,116,899.

No Drawing.

Application filed April 11, 1914. Serial No. 881,202.

To all whom it may concern:

Be it known that I, LEWIS B. LINDEMUTH, a citizen of the United States of America, residing at Steelton, in the county of Dauphin and State of Pennsylvania, have invented certain new and useful Improvements in Methods of Making Sound Steel Castings; and I do hereby declare the following to be a full, clear, and exact description of the invention, such as will enable others skilled in the art to which it appertains to make and use the same.

This invention relates to a method of making sound ingots or castings of steel, and has for its object to eliminate the pipe at the center of large bodies of metal, due to their natural cooling.

The method consists in placing on top of the ingot or casting, after it has been poured, a combustible in the form of a metalloid that has a high heat of combustion and which also, when oxidized, will not enter into the steel and change its composition. That is to say, I use a substance that develops a high heat, upon oxidation when placed upon the surface of the hot metal under the action of an oxidizing blast, and which is a metalloid in the sense that it is capable of acting both as an acid and a base. These substances are, silicon, which is preferably in the form of ferro-silicon, metallic aluminum, or titanium preferably in the form of ferro-titanium, which when free to oxidize are prone to slag formation rather than combination with or solution in the iron, so that they will not enter the metal at all, or at least, under most unfavorable conditions of use, will enter only about an inch into the surface portion of the metal that becomes agitated by the oxidizing blast. The substances I use have a specific gravity less than that of molten iron. The heat of combustion supplies the heat required to maintain the top of the casting molten until after the body of the casting has set sufficiently to overcome any tendency to form a pipe.

The material used according to this process with uniform success on a large number of ingots and other heavy castings, is silicon, preferably in the form of ferro-silicon containing fifty per cent. silicon, to which was supplied a blast of air under pressure, supplied through a half-inch pipe over the surface of the casting, the pressure of the air being sufficient to slightly agitate the

surface of the metal. The ferro-silicon is added from time to time, preferably in small lumps from one to three inches in diameter.

The heat developed is sufficient to keep the top of the casting in a fluid condition and at a high temperature.

In order to ascertain whether any of the silicon enters the metal, a large number of tests have been made, and samples of molten metal taken from an ingot at about the middle of the process show no appreciable change in composition of the steel, the analyses showing in some cases an increase of silicon of about three one-hundredths of one per cent. In making these tests a short crop end is cut off, not over 15% of the ingot; and numerous analyses at the point of severance show remarkable uniformity of the metal and normal silicon content.

It has heretofore been proposed to use carbon with a blast of air on top of an ingot, to prevent piping, but the carbon enters the steel and changes its composition, so that a great deal more metal will have to be cut from the top of the ingot. It has also been proposed to employ a blast of air only on the top of the metal, which is to combine with the silicon in the metal to produce the necessary heat; such an operation would rob the steel of its normal silicon content, so that this process also requires an abnormal amount of metal to be cut off at the top of the ingot to obtain an ingot of uniform composition throughout.

This invention is carried out as follows when used in connection with seven and a half ton ingots, twenty-six inches square and about seventy-eight inches long. The steel is teemed, either through the top or through the bottom of the ingot mold, and when the mold is nearly full and the metal is still rising in the mold, the air blast is turned on, on top of the metal with just sufficient force to agitate the surface. Immediately after the pouring of the metal has stopped a small quantity of ferro-silicon is thrown on top of the steel, and as the silicon is oxidized, more ferro-silicon is added from time to time, according to the appearance of the metal under the air jet, to keep up the temperature of the metal, and keep the top molten. As the slag increases the blast of air must be increased, in order to keep about three or four square inches, more or less, of the metal exposed to view. Roughly speaking, it takes about

five pounds of ferro-silicon per ton of ingot, and the operation continues an hour, more or less, until the body of the ingot has cooled sufficiently to obviate any tendency to pipe. The steel when teemed, is in a state known as "dead."

I claim—

1. The method of making sound castings, which comprises acting on the surface of the molten metal of the casting, until the body of the casting has solidified, with an oxidizing blast and a solid combustible that will not substantially enter the metal, said blast oxidizing the combustible as it melts.
- 15 2. The method of making sound steel castings which comprises acting on the surface of the molten metal, after teeming, and until the body of the casting has cooled sufficiently to prevent piping, with an air blast and a metalloid that is oxidized by the blast as it melts, will supply heat to the casting and will not substantially enter the molten metal.
- 20 3. The method of making sound castings, which comprises supplying an air blast and silicon to the molten surface of the casting after teeming and while cooling down sufficiently to prevent piping.
- 25 4. The method of making sound castings, which comprises supplying an air blast and ferro-silicon from time to time to the surface of the casting, during the cooling down of the casting sufficient to prevent piping.
- 30 5. The method of making sound castings, which comprises acting on the top of the molten metal with an oxidizing blast of suf-

ficient strength to keep a portion of the surface exposed and free from slag, and a substance that has a high heat of oxidation, is prone to slag formation and will not enter or substantially enter the metal of the casting and until the body of the casting has set or hardened, thereby keeping the surface portion of the casting molten, and preventing piping.

40 6. The method of making sound castings, which comprises acting on the surface of the molten metal of the casting with an air blast of sufficient strength to keep a portion of the surface exposed and free from slag, and adding ferro-silicon from time to time to keep the upper portion of the casting molten until the body of the casting has set or hardened, thereby preventing piping without causing the silicon to enter or substantially enter the metal.

45 7. The method of making sound steel castings, which comprises acting upon the surface of the molten steel while in the mold, until the body of the casting has solidified, with an oxidizing blast and a combustible that will not substantially enter the steel, thereby producing a solid steel casting of substantially uniform composition.

50 In testimony that I claim the foregoing as my invention, I have signed my name in presence of two subscribing witnesses.

55 LEWIS B. LINDEMUTH.

Witnesses:

CHAS. R. HOLTON,  
Wm. R. MILLER.